

April 26, 1949.

P. G. BRUNDELL ET AL  
PROCESS OF OBTAINING METALS, OXIDES, AND  
SALTS, FROM BITUMINOUS SHALE  
Filed Jan. 20, 1947

2,468,654



INVENTORS

Per Gunnar Brundell  
Stig Harald Tjernström

By:

Henry C. Parker Atty.

## UNITED STATES PATENT OFFICE

2,468,654

PROCESS OF OBTAINING METALS, OXIDES,  
AND SALTS, FROM BITUMINOUS SHALEPer Gunnar Brundell and Stig Harald  
Tjernström, Vargon, SwedenApplication January 20, 1947, Serial No. 723,202  
In Sweden June 29, 1943

18 Claims. (Cl. 75—30)

1

The present invention relates to a process of obtaining rare metals such as vanadium, molybdenum, titanium, tungsten and others, as well as iron and possibly also aluminium and potassium values from bituminous shale. A further object of the invention is to obtain a slag in the course of the process, which is readily transformable into slag-wool and similar valuable products. By the expression "bituminous shale" in this connection is meant an argillaceous rock impregnated by organic matter in the form of graphite, carbon and/or bituminous matter. As examples of bituminous shales there may be mentioned the alum shales belonging to the Upper Cambrian and the Lower Ordovician formations, which are found in quite heavy layers e. g. on the North American continent, in Scandinavia, Scotland, on the European continent and other places. The bituminous shale has for a long time been used for a number of technical purposes, e. g. as a fuel in the burning of lime, for production of shale oil and for the manufacture of building and insulating materials. Shales rich in alumina and potash have been used for the production of alum etc. It is also known that the bituminous shale often contains small percentages of such valuable metals as V, Mo, Ti, W and others. The content of these metals varies very strongly with the character of the shale. Thus, for instance, the Dictyonema shale frequently contains up to 0.35%, and sometimes even more, of vanadium, while molybdenum and tungsten are generally present only in quantities up to a few hundredths of one percent.

It has previously been tried to extract the vanadium content from the shale in a number of ways, e. g. by leaching with sulfuric acid, by froth-flotation, etc. The present invention is based on a new principle for treating shale with the object of obtaining valuable metals and compounds therefrom.

The following table is an example of frequently occurring average compositions of bituminous shales which may suitably be treated according to the invention.

|                                | Per cent |     | Per cent |
|--------------------------------|----------|-----|----------|
| Oil                            | 0-8      | MgO | 0-2      |
| C                              | 7-25     | S   | 2-10     |
| SiO <sub>2</sub>               | 45-55    | Fe  | 3-9      |
| Al <sub>2</sub> O <sub>3</sub> | 10-17    | Ti  | 0.3-0.6  |
| K <sub>2</sub> O               | 4-5      | V   | 0.04-0.4 |
| Na <sub>2</sub> O              | 0-1      | Mo  | 0-0.02   |
| CaO                            | 0-5      | W   | 0-0.01   |

If the carbon-containing shale is smelted, e. g. in an electric furnace, the carbon will reduce the

metal compounds present, so that a metal bath, the chief constituent of which is iron, and a siliceous slag floating on top of this are obtained. Our investigations have demonstrated that it is possible to cause the valuable metals such as V, Mo, W etc. to enter into this metal bath. The yield of e. g. vanadium, i. e. the proportion between the quantity of vanadium transferred to the metal bath and the total amount introduced in the furnace with the shale will, however, vary considerably owing to the conditions under which the process is carried out. Our investigations have demonstrated that the amount of metal obtained by this reduction process will, up to a certain limit, increase by decreasing carbon content in the raw material. This rather surprising result is explained by the fact that the amount of carbon present in the shale is considerably higher from the outset than what is necessary for obtaining a complete reduction of the metals in question. The excess carbon will cause considerable difficulties in the smelting of the shale since it will cause a reduction of the compounds contained in the siliceous slag. The products thus formed—chiefly silicon—will partly dissolve in the metal bath. At the same time considerable amounts will escape in a gaseous state from the furnace. This entails the formation of less favorable equilibria in regard to the yield of vanadium. Only in such cases where the chief object would be to obtain alumina and potash in the process would such a far going reduction of the siliceous matter be of any advantage, since by these expedients the silica content of the siliceous slag will be lowered, which makes the slag more suitable for leaching with acids to obtain salts of Al<sub>2</sub>O<sub>3</sub> and K<sub>2</sub>O.

Our investigations have thus demonstrated that if a high yield of e. g. vanadium is desired, the raw material, i. e. the shale should, previous to being fused, be subjected to a preparatory heating to oxidizing temperatures in the presence of air. This will lower not only the carbon content of the shale, but the non-oxidized (sulfide) sulfur content as well, a fact which has proven advantageous for the subsequent smelting.

According to the invention the shale material is thus subjected to a roasting or sintering in the presence of air previous to the reducing smelting, in order to lower its sulfidic sulfur i. e. its non-oxidized sulfur content. Such a roasting or burning is sometimes made in connection with known processes for recovery of oil from the shale, for which reason the solid residue

from such processes, e. g. the so-called shale-ash, in many cases is suitable for a direct use in the fusion process according to the invention.

The importance of lowering the sulfidic sulfur content in the material previous to the reducing smelting has been clearly demonstrated by our investigations. Ordinary bituminous shale of the kind particularly intended for processing according to the invention often has a sulphur content of from 2.5% to as high as 10%. Our investigations have demonstrated that considerable quantities of iron and vanadium (and in proportion also other valuable metals contained in the original shale) will remain in the slag, in spite of suitable adjustment of the carbon and CaO contents in the charge and in spite of sufficiently high reduction temperature, if the sulphur content of the ingoing shale material is comparatively high, and that a considerable increase in the yield is attained when, ceteris paribus, the sulfidic sulfur content in the material is lowered by oxidation previous to the reduction process.

The following figures may serve as an example of this significance. The figures relate to two samples of roasted shale having practically the same content of Fe, C and V and fused with the same amount of CaO; the difference mainly being in the sulfur content of the material.

| Charge | Fe       | S        | C        | V        | CaO-addition |
|--------|----------|----------|----------|----------|--------------|
|        | Per cent | Per cent | Per cent | Per cent | Per cent     |
| A----- | 4.7      | 1.0      | 3.4      | 0.29     | 20           |
| B----- | 4.5      | 2.0      | 3.3      | 0.29     | 20           |

Contents in the corresponding slags.

| Slag from | FeO      | S        | CaO      | V        | SiO <sub>2</sub> |
|-----------|----------|----------|----------|----------|------------------|
|           | Per cent | Per cent | Per cent | Per cent | Per cent         |
| A-----    | 0.6      | 1.0      | 21       | 0.03     | 53               |
| B-----    | 2.9      | 1.6      | 23       | 0.19     | 52               |

Yield of vanadium as metal.

| From charge | Yield    |
|-------------|----------|
|             | Per cent |
| A-----      | 89       |
| B-----      | 31       |

The difference in the result at different sulphur contents is striking. Since in this case it was the question of two shale materials which had been de-sulfurized to a different degree by a differently strong roasting, it is evident that the effect of the lowering of the sulfur content must be still more pronounced when comparing our process with smelting processes in which a shale material is subjected to a reducing smelting without any previous roasting or oxidation at all and which for this reason has a still higher sulphur content.

When reference is made to the sulphur content it should always be remembered that it is here a question of the non-oxidized, i. e. the sulfidic sulfur. If the roasting is, for instance, carried out on the shale when mixed with lime or limestone, the sulfur may to a great extent be retained by the lime in the form of sulfite or sulfate. Analytically the sulfur content of the charge may thus appear to remain high, but due

to the oxidation which the sulfur has undergone during the roasting it no longer appears in its sulfidic form and has thereby lost its detrimental effect on the metal yield in the reduction process, as our investigations have demonstrated. A plausible explanation of our discovery that the sulfidic sulfur in the shale should be brought below 1.5% and suitably under 1% to obtain satisfactory yields of metals is that the sulfur in the shale is chiefly bound to the metals in a sulfidic state. Thus the iron—at least for the main part—is present as pyrite and the vanadium probably as V<sub>2</sub>S<sub>3</sub>. If such a shale material having a comparatively high sulfur content, which for instance in Dictyonema shale is often around 2.5–4%, is directly subjected to a reducing smelting, the resulting poor yield most likely may be attributed to a formation of a finely dispersed sulfidic matte which retains a large part of the metals in the slag instead of letting them pass over into the metallic bath. If the shale contains oil this may of course first be recovered by known methods, previous to a lowering of the carbon content of the material by burning.

We have found that by burning out the carbon in the shale or its distillation residue to such a degree that the amount of carbon left in the shale is within the range of from one to five times

the amount theoretically needed for a reduction of all the content of Fe<sub>2</sub>O<sub>3</sub>, TiO<sub>2</sub>, V<sub>2</sub>O<sub>5</sub>, MoO<sub>3</sub> and WO<sub>3</sub> to corresponding metals, exceedingly high yields of vanadium and other valuable metals may be realized. It is, of course, also possible to adjust the carbon content by mixing a shale, the carbon content of which is more or less completely burnt out, with a shale more rich in carbon or with some other suitable carbonaceous material, e. g. coal or coke, so that the above mentioned desired proportions of from one to five times the theoretical

amount of carbon needed for a reduction of the above mentioned oxides is obtained in the charge. Such additional reduction agent may also, instead of in the form of carbonaceous material, be added in the form of e. g. FeSi, CaSi, CaC<sub>2</sub>, Si, Al, Mg,

reducing gases, such as H<sub>2</sub>, producer gas and similar. It may also be advantageous to adjust the carbon content by adding reducible oxides or similar material e. g. iron ore or other iron containing materials, whereby a simultaneous ad-

justing of the amount of vanadium and if desired also of molybdenum and tungsten in the resulting metal bath may be obtained. It should, however, be noted that the carbon or carbonaceous material which is naturally present in the shale occurs in

a highly intimate mixture with the other components, and for this reason this carbon shows a better reducing action than such reducing agents which are added to the charge.

As already stated, it is thus by a suitable proportioning of the reducing agent, in particular the carbon contained in the shale, possible to realize a considerable improvement in the yields of the metals vanadium, molybdenum etc. By this expedient the advantage is also obtained that the energy-consuming reduction of the silica in the shale is highly depressed.

The equilibrium between slag and metal bath is also to a higher or lesser degree influenced by other factors. Thus our tests have shown that changes in the acidity of the slag may cause great variations in the yield of vanadium, molybdenum etc. A suggested explanation of this is the amphoteric nature of the corresponding metal oxides although nothing definite can be said as to the reasons for the stated and ob-

served fact. The acidity of the slag may be adjusted by the addition of basic slag forming material. By this addition the fusing point of the slag is influenced in the sense that it falls with rising content of basic material. Hereby it is possible to attain the temperature range which is most favorable for the reduction process. At too high reduction temperatures, e. g. when the slag has a high fusing point, the yield of vanadium will decrease at the same time as the iron content of the slag increases. At too low reduction temperatures, on the other hand, the reduction will become unsatisfactory. It is thus possible to adjust the reaction conditions properly by adjusting the acidity (basicity) of the slag, which stands in close relation to its fusing point. Suitable reaction conditions are as a rule obtained within the temperature range 1500° to 1800° C., particularly in the vicinity of 1600° C..

If the shale is melted together with a suitable amount of burnt lime, limestone, dolomite and/or other slag forming basic materials containing CaO, MgO, BaO, Na<sub>2</sub>O or K<sub>2</sub>O the yield of vanadium, molybdenum etc. may thus be considerably increased. The addition of burnt lime, limestone or equivalent basic material, which necessarily must be adjusted with regard to the composition of the shale, will thus vary between wide limits. The addition, however, must be sufficient to produce a lowering in the viscosity of the slag but not substantially exceeding the quantity required to produce a basicity in the slag bath corresponding to a CaO content of up to 60%. The optimum conditions are, however, generally obtained in the rather narrow range of about 10 to 25% CaO. Additions of lime or other basic material in such quantities that the basicity of the slag will be over 60% calculated as CaO, entails a gradually increasing and undesirable formation of carbides. The viscosity curve will also become of such form that the slag will be unsuitable for slag-wool production.

The favorable influence of the basic addition on the yield of vanadium etc. is that it makes the slag more fluid, by lowering its viscosity, whereby a more rapid separation of slag and metal may be effected, tapping is facilitated and better conditions will prevail during the smelting, since the heat transfer in the molten charge is considerably improved when the slag is easy flowing. When utilizing the slag for making slag-wool and similar products a still lower viscosity than what is produced within the above mentioned optimum basicity range may be desirable in order to obtain a suitable composition and workability of the slag for said purpose. In such event the basicity, computed as CaO, may suitably be increased up to as high as 40% and even more. This will generally mean a slight decline in the yield of vanadium which, however, in such cases is more than offset by the gain in regard to the quality of the slag, since the removal of iron from the slag will be practically unchanged while the physical properties desirable in slag-wool products are materially improved.

Our investigations have demonstrated that it is of great importance that the slag forming basic materials are added in the right proportions. Thus the yield of vanadium, molybdenum etc. will first increase with increased addition of basic material up to a maximum and then

again fall upon further increase of the basic components in the slag. It is, however, not possible to state any definite figure for the position of the maximum point that would hold for general conditions, because of the rather complicated system which is represented by the slag. It is evident that the maximum point will become displaced according to the composition of the shale, the largest variations being due to the contents of SiO<sub>2</sub>, Al<sub>2</sub>O<sub>3</sub> and alkali in the shale. The aforementioned figures for the slag basicity, corresponding to not over 60% calculated as CaO and preferably lying between 10 to 25% CaO will, however, hold for the usual composition of the shales e. g. as according to the above stated table of analysis.

The heat value of bituminous shale is generally between 500 and 2500 kilogram calories per kilogram. When adjusting the carbon content of the shale according to the invention, a considerable amount of the heat value of the material may be utilized by calcining a quantity of limestone with the aid of the burning shale, said quantity being calculated such that the mixture of burnt lime and shale ashes resulting from the burning will yield a siliceous slag in the subsequent smelting, having a suitable CaO-content for obtaining the highest yield of vanadium. For shales with higher heat values the burning may be carried out in such a manner that the mixture of shale ashes and burnt lime will leave the furnace with a temperature of up to 950° C. or more, in which condition the mixture is ready for immediate charging into an electric furnace. The burning and preheating may of course also be aided by addition of suitable fuels, e. g. coke. The smelting process is not limited to the use of electric furnaces but may also be carried out in blast-furnaces, reverberatory furnaces or the like.

While testing various modes of carrying out the oxidizing step of the invention we have made the rather surprising discovery that the use of a sintering process similar to the known procedures for treating metal ore concentrates and employing similar equipment, e. g. as described in Liddel "Handbook of Non-Ferrous Metallurgy" (part I, 1945, Chapter X, Roasting and Sintering), produces very favorable results in several respects as against conventional roasting treatment, as will be more fully explained in the following.

Previous to such sintering the charge is reduced to a suitable particle size. If it is desired to obtain a sinter with good mechanical strength for the purpose of being used in smelting equipment where such strength is desirable, the crushing of the shale and other material possibly entering the charge, should preferably be made so that the various grain classes will be fairly uniformly present. A suitable grading is generally obtained by crushing down the raw-material to correspond to a maximum of about 5 millimeters in diameter. In order to prevent clogging finer grains than about 0.08 millimeters should be avoided.

The ignition of the sintering charge is made in the same manner as known in connection with the conventional sintering of metal ore concentrates, e. g. by means of a gas-burner or by using a layer of charcoal breeze and wood-wool. In order to lower the resistance for the suction of gases through the charge during sintering, this is suitably "loosened up" or made porous by

means of an addition of water in an amount of for instance 5-15 per cent of the weight of the charge. The charging of the sintering pan is suitably made over a spike roller or through a screen to preserve the even and porous structure of the charge when placed in the pan.

The shale material employed has generally such a high heat value that no extra fuel is needed in the charge. On the contrary, there is frequently so much fuel contained in the shale material that considerable quantities of basic slag forming substances may be admixed therewith without the heat value becoming too low. Thus, for instance, in sintering a shale containing 9% C, an addition of up to 70% of the weight of the shale of limestone, dolomite or other suitable carbonate containing material may be made, whereby these carbonate materials at the same time will for the larger part become transformed to oxides. In this manner it is possible in a very simple way to produce a charge which after a possible addition of reducing agents is ready for immediate use in the smelting furnace.

Our tests have shown that if the shale particles exceed a certain grain size, which however varies somewhat with the nature of the material, they will not become completely roasted but will contain an unroasted core. By adjusting the grain size it is thus by means of a few test-runs possible to determine how much carbonaceous material may be left in the sinter to be used as reducing agent in the following smelting process. The amount of carbon which in this manner may be left, is however dependent on how far the simultaneous oxidation and removal of the sulfide sulfur can be realized, as this varies from one shale to another. In some instances it is necessary to burn out practically all of the carbon in the shale in order to lower the sulfide sulfur to an amount corresponding to optimum yield of metals in the subsequent reduction process. Other shales on the other hand, when roasted down to a carbon content of about 3% which is suitable for the reduction process, have at the same time lost enough sulfide sulfur to suit the optimum requirements, and no extra reduction agent is thus needed in such cases.

As already mentioned in the foregoing, a roasting in the presence of basic slag forming materials, e. g. limestone, may cause the sulfur originally contained as unoxidized sulfide sulfur in the shale to remain for the larger part in the charge, although now in the form of sulfite and sulfate and thus without detrimental influence on the subsequent metal reduction process. We have found that some of these sulfites and sulfates may become thermally dissociated whereby sulfur partly escapes in the form of oxides and partly is reduced back to a sulfidic form. This "secondary" sulfide sulfur is, however, of no detrimental influence on the yield of e. g. vanadium, since the sulfur in this case during the reduction is bound to the lime. By increasing the sintering temperature for instance from 950° C. to 1200° C., e. g. by increasing the heat value of the charge, using stronger suction through the pan, etc. it will thus, owing to a higher thermal dissociation of the sulfites and sulfates already during the sintering operation be possible to cause a substantial lowering of the total sulfur content of the charge. This will materially help to lessen the formation of "secondary" sulfide sulfur in the subsequent reduction process which, even if it is of no particular value in regard to

the yield of metal, is of importance in making slag-wool or "foam" by conventional methods from the ensuing slag. Already a fraction of a percent of calcium sulfide in the product may be sufficient to spoil its quality, owing to the instability of this compound under certain conditions particularly in the presence of Fe. Such a sintering temperature that thermal dissociation of sulfites and sulfates will take place to a substantial degree is thus a valuable step in the process according to the invention. Especially in the case of slag "foam," where the material contains numerous pores and vesicles in which hydrogen sulfide, which may form when the calcium sulfide in the slag is brought in contact with water during the well known "foaming" process, becomes included and from which it subsequently gradually diffuses into the atmosphere, it is extremely important that the product is as stable as possible, since it will otherwise be perfectly valueless as insulating material in buildings because of its nauseating smell.

When sintering is made of a charge having a very high heat value, a fusing may take place in the sintering zone. The grains of shale material in the charge will thereby become encased in an impervious glazing and prevented from becoming roasted or oxidized. This may be prevented by adjusting the heat value of the charge by adding a sufficient amount of "returns" from previous sinterings in the ingoing charge on the sintering equipment.

If the sintering operation is interrupted when the zone of sintering has reached the grate the sinter generally is very hot (e. g. 500°-800° C.). From the point of heat economy it is advantageous to charge this hot sinter directly into the reduction furnace, possibly after a coarse crushing.

The high efficiency of the process in transferring the metals in question into the metal bath entails the great advantage that the slag will show a comparatively low content of the sulfide forming heavy metals in question (Fe, V, Mo, W); the percentage of Fe being generally below 0.5% and quite frequently as low as 0.2%, the other metals (V, Mo, W) in proportion thereto generally being present in a total quantity of less than 0.05%. When blowing such slag by known methods a slag-wool of light color and very attractive appearance is obtained, provided that the basicity is sufficiently high e. g. 25-45% ad even up to 55% calculated as CaO. A far going reduction of the heavy metals (Fe, V, Mo etc.) is very much dependent upon the degree to which the corresponding sulfides are transferred to oxides during the sintering. A reducing smelting of shale or shale residue having a high content of sulfide sulfur bound to heavy metals will yield a slag which contains a comparatively high percentage of these metal sulfides in solution or very finely dispersed. A slag wool from such a slag will have a dark color and frequently decomposes in the presence of moisture while giving off sulfur containing gases.

As an example of the result of a properly conducted sintering according to above stated principles may be mentioned that a slag-wool blown from a slag which had a content of "secondary" sulfide sulfur as high as 1.7% (chiefly as calcium sulfide) but practically free from heavy metals (0.3%) upon boiling in water for 6 hours did not lose more than 0.0009% S.

The invention can be understood readily from

a study of the accompanying drawing in which the figure is a flow sheet of our process. The legends on this flow sheet are believed to make it self explanatory.

In the flow sheet the arrows shown in full lines represent the preferred procedures while those with dotted stems represent optional procedures. As indicated, a charge of bituminous shale is first subjected to an oxidizing treatment which may be either a roasting or a sintering procedure. The conditions are so controlled during the oxidation that the sulfidic sulfur content is reduced below 1.5%. Limestone or dolomite can be added to the charge undergoing oxidation if desired. The reducing agent content of the resulting shale ash is then controlled so that the reducing agent present amounts to from about 1 to 5 times that required to reduce the metal oxides. The lime content is also controlled so that the reducing agent present amounts to from about 1 to 5 times that required to reduce the metal oxides. The lime content is also controlled so that from 10 to 60% by weight is present. The batch is then smelted. The slag is drawn off and either blown into slag wool or treated for recovery of its  $Al_2O_3$  and  $K_2O$  contents. The metal which is recovered from the smelting step contains substantially the entire content of vanadium, molybdenum, tungsten and titanium present in the original bituminous shale.

Our invention can be explained in greater detail by reference to the following specific examples which represent practical operating embodiments of processes which result in the recovery of metal values and slag wool from bituminous shales in accordance with the present invention. These examples are not to be considered as limiting the scope of our invention.

#### EXAMPLE 1

1000 kilograms of shale containing 9% C and 2.6% S (as sulfides) were crushed down in a ball mill to a maximum particle size of 3 millimeters with an even grain class distribution down to about zero and mixed with 700 kilograms of dolomite (all particles below 3 mm. and about same grain distribution as the shale). The mixture was moistened with 225 kilograms of water and subjected to sintering in an ordinary suction sintering pan. The sintering temperature was during the operation which lasted 30 minutes kept around  $950^{\circ}C$ . The highest temperature of the escaping gases was  $220^{\circ}C$ . No extra fuel was added.

The resulting sinter contained 0.1% C, 0.2% sulfide-S, 19.2% CaO and 13.2% MgO. The total sulfur content of the sinter was 1.2%. After reducing smelting for recovery of metals according to the previously described procedure in a direct arc furnace the slag was recovered and blown to wool by the conventional method using compressed air as blowing medium. The wool product showed very high quality in regard to color and elasticity. It analysed as follows:

|               | Percent        |
|---------------|----------------|
| $SiO_2$       | 45.0           |
| $Al_2O_3$     | 13.7           |
| $TiO_2$       | 0.4            |
| CaO           | 20.3           |
| MgO           | 14.5           |
| Fe            | 0.2            |
| V, Mo         | Less than 0.04 |
| S             | 1.0            |
| Alkali oxides | 4.1            |

The yield of vanadium was in this instant 89% in spite of the fairly high basicity of the slag, which demonstrates the efficiency of the sintering process as applied in our invention.

5 The surprising discovery in the course of our investigations, that the heating of the raw-material while subjecting it to oxidizing conditions, with or without the presence of additions of basic slag forming substances, to such high temperatures that a sintering takes place which at first was considered objectionable, instead produces a charging material for the reduction step in the process which is exceedingly apt to give high yields of metals under such conditions that a 10 slag is at the same time obtained which is particularly well suited to be worked up to slag-wool and similar products, means a very definite improvement both of a technical and commercial 15 nature of our process as originally outlined. The 20 sintering procedure not only facilitates the proper adjustment of the carbon content in the oxidized material intended for the subsequent reduction step, at the same time as it permits of a very far going oxidation of the sulfur, but it also provides 25 a material which in the reduction step readily lends itself to a quite unexpected completeness of separation of the heavy metals in the charge into the metal bath while leaving a very pure slag behind. The reason for this favorable result is not quite understood but we at least partly attribute it to the very even oxidation of the 30 raw-material which may be obtained in a sintering apparatus as against other conventional shale roasting or burning equipment, such as shaft-furnaces and the like, as well as possibly to the 35 more even distribution of the homogeneously oxidized shale material in the charge which is attained in this manner, particularly when the sintering procedure is carried out with a mixture 40 also containing basic slag forming additions, in which case a very uniform charging material for the reduction furnace is obtained, whereby the chemical reactions and the separation of the slag and metals evidently is highly facilitated.

45 As further representative examples of sintering procedures according to the invention the following may be stated.

#### EXAMPLE 2

50

| Charge          | Kilo-<br>grams | Total<br>S  | Sub-<br>fide S | C           | CaO         | MgO         |
|-----------------|----------------|-------------|----------------|-------------|-------------|-------------|
|                 |                | Per<br>Cent | Per<br>Cent    | Per<br>Cent | Per<br>Cent | Per<br>Cent |
| Shale           | 925            | 2.6         | 2.6            | 9           | -----       | -----       |
| Dolomite        | 500            | -----       | -----          | -----       | -----       | -----       |
| Water           | 125            | -----       | -----          | -----       | -----       | -----       |
| Obtained sinter | -----          | 0.8         | 0.3            | 0.2         | 19.2        | 12.2        |

60 The charge which had the same grain class distribution as in Example 1 was treated in the sintering apparatus without extra fuel, except for the ignition. The operation lasted for 45 minutes during which time the oxidation and sintering took place. The maximum temperature in the sintering zone was about  $1000^{\circ}C$ . The obtained sinter was crushed to lumps of about 2" diameter and mixed with 4.5 per cent of its weight of charcoal breeze ( $\frac{1}{2}$ " lumps). The well 65 mixed charge was then smelted in a direct arc electric furnace. The slag was tapped at about  $1500^{\circ}C$ . and blown to slag-wool by means of compressed air in the conventional way whereby a 70 product with long, fine glass-wool like, extremely 75 elastic fibres was obtained.

The metal bath was recovered separately and cast to ingots. The yield of vanadium was 89%. The slag analyzed:

|                                | Percent |
|--------------------------------|---------|
| SiO <sub>2</sub>               | 44.2    |
| Al <sub>2</sub> O <sub>3</sub> | 11.8    |
| TiO <sub>2</sub>               | 0.4     |
| CaO                            | 22.5    |
| MgO                            | 14.2    |
| Fe                             | 0.3     |
| V, Mo                          | 0.03    |
| S                              | 0.8     |
| Alkali oxides                  | 4.8     |

## EXAMPLE 3

| Charge          | Kilo-<br>grams | Total S         | Sulfide<br>S    | C             | CaO      | MgO      |
|-----------------|----------------|-----------------|-----------------|---------------|----------|----------|
| Shale           | 700            | Per cent<br>2.6 | Per cent<br>2.6 | Per cent<br>9 | Per cent | Per cent |
| Returned sinter | 800            | 0.7             | 0.2             | 0.3           | 0.2      | -----    |
| Water           | 180            | 0.7             | 0.2             | 0.3           | 2.1      | 1.6      |
| Obtained sinter | -----          | -----           | -----           | -----         | -----    | -----    |

The sintering operation was mainly carried out as described in connection with Example 2, the grain sizes of the material being about the same. The main difference from Example 2 is that no carbonate material (dolomite, limestone) was added. For this reason a certain quantity of ready sinter was returned and mixed with the charge, as seen from the table, in order to adjust the mean heat value of this, which otherwise would have been too high. The obtained sinter was reduced to lumps of about 2" diameter and mixed with 45 per cent of its weight burnt lime and 5.5 per cent of its weight coke breeze (below  $\frac{1}{4}$ ").

The charge was smelted as in Example 2. Yield of vanadium 87%. The basic content of the slag calculated as CaO was 39%. The slightly lower yield of vanadium as against Example 2 is probably mainly due to the fact that the sintering took place in the absence of basic additions. In all three examples the amount of reducing agent in the fusing step was about two to three times that needed for reduction of the heavy metal oxides.

The slag-wool obtained according to the invention is in its general appearance of about the same character as glass-wool, i. e. it differs favorably from other known slag-wool and so called rock-wool products in that it has considerably longer fibres, which even compared to glass-wool show a great improvement as regards elasticity. The product is easily distinguished from all of the aforementioned known products by its chemical analysis, the characteristic features of which are as follows:

|                                     |                                    |
|-------------------------------------|------------------------------------|
| Fe                                  | Below 0.5%                         |
| S                                   | 0.3% to 2.0%, normally<br>about 1% |
| Total CaO, MgO and<br>alkali oxides | 25% to 55%                         |
| Alkali oxides                       | 2%-7%, normally 4%-5%              |
| SiO <sub>2</sub>                    | 38%-50%                            |
| Al <sub>2</sub> O <sub>3</sub>      | 10%-15%                            |

The slag may to advantage be used not only for producing slag-wool by known methods but also other products such as "slag-foam" and similar insulating materials, owing to its high qualities in regard to properties desirable in the manufacture and use of these known products.

The siliceous slag may also be finely ground and leached with acids in order to obtain aluminium

and potassium values. The facility of extraction increases strongly and rapidly with increased basicity of the slag, so that it is possible already at a comparatively low basicity, within the limits stated, to obtain a practically complete recovery of said values.

From what has been stated above is seen that the process according to the invention will give extremely high yields of vanadium and other valuable metals when observing the conditions in regard to proper adjustment of the carbon content of the shale and in the charge, a lowering of heavy metal bound unoxidized sulfur prior to smelting to below 1.5% and preferably below 1%,

adjusting the basicity of the slag etc. Our tests have shown that it is possible to attain an almost quantitative collection of such metals as V, Mo, Ti and W in the metal bath if these conditions are properly observed, i. e. by smelting shale with a suitable carbon content together with the proper amount of lime, according to the general principles of the invention already set forth. As already mentioned, the siliceous slag obtained in the process is well suited to a further treatment for the obtaining of Al<sub>2</sub>O<sub>3</sub> and K<sub>2</sub>O therefrom, as well as for the manufacture of building and insulating materials.

It should in this connection be pointed out that in order to sufficiently lower the original sulfide sulfur content it may be necessary to subject the shale to such an intense oxidizing treatment that its inherent carbon content may be burnt down to such extent that addition of external reduction agent is necessary. The above outlined sintering procedure has in these instances proven particularly useful for preparing a shale material which will readily lend itself to complete reduction in regard to the metals in question in spite of the fact that use can not be had of "native" carbon in the shale except to perhaps a very small extent. This is probably due to the fact that a sintered charge becomes very porous whereby a gas-transport into it from external reduction agents is facilitated.

The slag and metal baths may be tapped from the furnace either separately or together, in which latter case they are separated outside this and subsequently treated separately.

The metal bath obtained by the smelting, will in favorable cases hold e. g. 10% vanadium and may be processed in various ways, for instance by forming a vanadium slag by adding iron ore, chromium ore or other suitable ore. The remaining iron may to advantage be worked up to steel e. g. in an electric steel furnace.

Considering the fact that the percentages of vanadium, molybdenum etc. in the shale are very small and in general of the same order of magnitude as those in slags from metallurgical processes, and furthermore considering that the slag bath constitutes about 90 to 110% and the metal bath only 10 to 5% of the shale raw material entering the process, it must be said to be quite surprising that under these circumstances it is possible to carry out a metallurgical process with an almost quantitative yield of the said metals. The reason for this extremely satisfactory result may, in addition to the above outlined expedients in regard to proper adjustment of the carbon and lime content, in such cases where only a mild roasting has taken place, be sought in the fact that at least a substantial proportion of the reducing agent employed consists of the carbon present in the material itself, which as already stated,

in the bituminous shales is intimately distributed

throughout the material, whereby an exceedingly even and speedy reduction is obtained.

The following examples serve to further illustrate the process according to the invention as applied without sintering.

A Dictyonema shale having an ignition loss of 18.1% contained 9.5% carbon and a 3.1% sulfur. After roasting this shale yielded an ash of the following composition:

|                                | Per cent | 10 |
|--------------------------------|----------|----|
| Ignition loss                  | 4.0      |    |
| SiO <sub>2</sub>               | 59.2     |    |
| Al <sub>2</sub> O <sub>3</sub> | 18.5     |    |
| Fe <sub>2</sub> O <sub>3</sub> | 6.7      |    |
| TiO <sub>2</sub>               | 0.5      | 15 |
| V <sub>2</sub> O <sub>5</sub>  | 0.6      |    |
| (V=0.318%)                     |          |    |
| P <sub>2</sub> O <sub>5</sub>  | 0.2      |    |
| CaO                            | 1.4      |    |
| MgO                            | 2.3      |    |
| K <sub>2</sub> O               | 5.0      | 20 |
| Na <sub>2</sub> O              | 1.5      |    |
| Carbon                         | 2.5      |    |
| Sulfur                         | 1.0      | 25 |

15,300 kg. of this ash was mixed with 2300 kg. of burnt lime with the following analysis:

|                                | Per cent |    |
|--------------------------------|----------|----|
| Ignition loss                  | 3.0      |    |
| SiO <sub>2</sub>               | 8.2      |    |
| Al <sub>2</sub> O <sub>3</sub> | 0.8      |    |
| Fe <sub>2</sub> O <sub>3</sub> | 0.7      |    |
| CaO                            | 84.8     | 30 |
| MgO                            | 2.3      |    |

The mixture was fused in an electric furnace. Hereby 15,200 kg. of slag and 849 kg. of metal were obtained with the following compositions:

| Slag:                          | Percent Metal: | Per cent |      |
|--------------------------------|----------------|----------|------|
| SiO <sub>2</sub>               | 57.7           | Fe       | 78.0 |
| Al <sub>2</sub> O <sub>3</sub> | 18.5           | Si       | 13.6 |
| Fe <sub>2</sub> O <sub>3</sub> | 0.5            | V        | 5.21 |
| TiO <sub>2</sub>               | 0.3            | Ti       | 1.5  |
| CaO                            | 14.1           | P        | 0.7  |
| MgO                            | 2.4            | Mo       | 0.25 |
| Alkalies                       | 6.4            | Mn       | 0.5  |
|                                | 99.9           |          | 99.8 |
|                                |                | Per cent |      |
| Sulfur                         | 0.8            |          | 60   |
| V                              | 0.029          |          |      |
| Vanadium yield                 | 91             |          |      |

As a further example of the efficiency of the process according to this embodiment of the invention may be stated that a shale ash with a vanadium content of 0.06% upon fusing with lime gave a vanadium yield of 96%.

The following tables demonstrate the influence of the carbon and lime contents. The starting materials consisted of burnt lime of above analysis and shale from which the above ash was prepared by roasting without sintering.

#### 1. VARIATIONS IN THE CARBON CONTENT

CaO-content of slag about 14%

| Carbon content in ash | Vanadium in Metal bath | Yield of vanadium |
|-----------------------|------------------------|-------------------|
| Per cent              | Per cent               | Per cent          |
| 1.2                   | 3.56                   | 61                |
| 2.0                   | 4.92                   | 85                |
| 2.5                   | 5.21                   | 91                |
| 3.4                   | 4.89                   | 88                |
| 8.2                   | 2.71                   | 28                |

#### 2. VARIATIONS IN THE LIME ADDITION

Carbon content of ash about 3.4%

| CaO-content of slag | Vanadium in metal bath | Yield of vanadium |
|---------------------|------------------------|-------------------|
| Per cent            | Per cent               | Per cent          |
| 2.0                 | 3.38                   | 65                |
| 9.3                 | 4.12                   | 77                |
| 14.0                | 4.89                   | 91                |
| 19.7                | 4.92                   | 90                |
| 25.5                | 4.56                   | 83                |

These figures are of particular interest when compared with the high yields of vanadium which are obtained in the upper basicity range, from about 25 to 45% CaO and more, when using a sintered charge and which as a rule can not be attained by a mere roasting of the material.

The present application is a continuation-in-part of our copending application, Serial No. 541,270, filed June 20, 1944, which now stands abandoned.

We claim:

1. In the treatment of bituminous shales by reducing smelting for recovery of at least one of the metals vanadium, molybdenum, titanium and tungsten contained therein, the process which comprises first heating such a shale to oxidizing temperatures in the presence of air under conditions causing a lowering of its heavy metal-bound sulfidic sulfur content to below 1.5 per cent by weight; adjusting the reducing agent content of the charge to be smelted to within the range from about 1 to 5 times the quantity required for complete reduction of the metal oxides of iron, titanium, vanadium, molybdenum and tungsten contained therein, adding basic, slag forming materials in quantity sufficient to lower the viscosity of the slag formed in the subsequent fusion step but not substantially exceeding the quantity required to produce a basicity in the slag bath corresponding to a quantity of 60 per cent by weight of said slag, calculated as CaO, fusing to form a metal bath and a siliceous slag bath, separating the metal bath and recovering the metal values therefrom.

2. A process for the recovery from solid bituminous shale distillation residue of at least one of the metals vanadium, molybdenum, titanium and tungsten contained therein by reducing smelting, comprising selecting such a material having a content of heavy metal-bound sulfidic sulfur of less than 1.5 per cent by weight, adjusting the reducing agent content of the charge to be smelted to within the range from about 1 to 5 times the quantity required for complete reduction of the metal oxides of iron, titanium, vanadium, molybdenum and tungsten contained therein, adding basic, slag forming materials in quantity sufficient to lower the viscosity of the slag formed in the subsequent fusion step but not substantially exceeding the quantity required to produce a basicity in the slag bath corresponding to a quantity of 60 per cent by weight of said slag, calculated as CaO, fusing to form a metal bath and a siliceous slag bath, separating the metal values therefrom.

3. The process according to claim 1 wherein the basicity of the slag is adjusted to within the range of from about 10 to 25 per cent by weight, calculated as CaO.

4. The process of claim 1 wherein the bitumi-

nous shale originally contains an excess of carbon, the carbon content being brought within the limits stated during the oxidizing treatment.

5. The process of claim 1 wherein the bituminous shale contains an excess of reducing agent and the relative quantity of the latter in the charge is adjusted by the addition of iron oxide.

6. The process of claim 1 wherein basic material necessary for adjusting the basicity of the slag is added in the form of carbonate previous to the oxidizing step whereby during the course of the oxidizing treatment it is transformed to the oxide state.

7. The process of claim 1 wherein the temperature in the oxidizing step is sufficient to cause a sintering of the material to be oxidized.

8. The process of claim 1 wherein the temperature in the oxidizing step is sufficient to cause a substantial thermal dissociation of the sulfur oxidation products formed.

9. The process of claim 1 wherein the basicity of the slag is adjusted to within the range of from 25 to 55 per cent by weight calculated as CaO, and wherein after separation from the metal bath said slag is transformed into a slag-wool product.

10. The process of claim 1 wherein the oxidizing and fusing steps are conducted in different equipment and the product obtained in the oxidizing step is transferred to the fusing step at high temperatures up to about 950° C.

11. In the treatment of bituminous shales by reducing smelting for recovery of at least one of the metals vanadium, molybdenum, titanium and tungsten contained therein, the process which comprises heating such a shale to oxidizing temperatures in the presence of air under conditions producing a lowering of its heavy metal-bound sulfidic sulfur content to below 1.5 per cent by weight, adding basic, slag forming materials in quantity sufficient to lower the viscosity of the slag formed in the subsequent fusion step but not substantially exceeding the quantity required to produce a basicity in the slag bath corresponding to a quantity of 60 per cent by weight of said slag, calculated as CaO, subjecting said mixture to a reducing smelting to form a metal bath and a siliceous slag bath, separating the metal bath and recovering the metal values therefrom.

12. In the treatment of bituminous shales for recovery of their vanadium, molybdenum and tungsten contents, the process which comprises adjusting the reducing agent and lime contents of such a shale so that the reducing agent content is insufficient to cause any substantial reduction of the SiO<sub>2</sub> present to Si in the subsequent fusion step and is from 1 to 5 times the quantity required for the complete reduction of the metal oxides of iron, titanium, vanadium, molybdenum and tungsten contained therein and the CaO content is within the range of about 10 to 25 per cent based on the weight of the siliceous slag-forming components, at least a substantial proportion of the reducing agent present consisting of the natural carbonaceous material in said shale, then fusing the mixture to form a metal bath and a siliceous slag bath, separating the metal bath from the slag bath and treating them separately for the recovery of their metal and mineral values.

13. The process of claim 12 wherein the reducing agent content of said slag is adjusted by roasting the bituminous shale to reduce its carbon content to within the range stated.

14. In the treatment of bituminous shales for

recovery of their vanadium, molybdenum and tungsten contents, the process which comprises adding limestone to such a shale in quantity sufficient to supply from about 10 to 25 per cent CaO by weight based on the weight of the siliceous slag-forming components present, roasting the mixture to calcine the limestone to CaO and to reduce the carbon content to within the range of about 1 to 5 times that required to produce complete reduction of the oxides of the metals iron, titanium, vanadium, molybdenum and tungsten which are present and insufficient to cause any substantial reduction of the SiO<sub>2</sub> content to Si in the following fusion step, then fusing the mixture to produce a metal bath and a siliceous slag, separating the metal bath and recovering metal values therefrom.

15. The process of claim 14 wherein the roasting and fusing steps are conducted in different furnaces and the mixture is transferred from the roasting to the fusing furnace at high temperatures not exceeding about 950° C.

16. In the treatment of bituminous shales for recovery of their vanadium, molybdenum and tungsten contents, the process which comprises roasting such a shale in the presence of air to lower its carbon content below that producing any substantial reduction of the SiO<sub>2</sub> present to Si in the following fusion step but leaving the carbon content within the range of from 1 to 5 times the quantity required for complete reduction of the metal oxides of iron, titanium, vanadium, molybdenum and tungsten contained therein, adjusting the content of basic, slag-forming materials in the shale to within the range of about 10 to 60 per cent, calculated as CaO, fusing to form a metal bath and a siliceous slag bath, separating the metal bath and recovering metal values therefrom.

17. In the treatment of bituminous shales for recovery of their vanadium, molybdenum and tungsten contents, the process which comprises roasting such a shale in the presence of air and adjusting its carbon content within the range of from about 1 to 5 times the quantity required for complete reduction of the metal oxides of iron, titanium, vanadium, molybdenum and tungsten contained therein, adding basic, slag-forming materials in quantity sufficient to lower the viscosity of the slag formed in the subsequent fusion step but not exceeding a quantity of 60 per cent by weight, calculated as CaO, fusing to form a metal bath and a siliceous slag bath, separating the metal bath and recovering metal values therefrom.

18. The process which comprises heating a bituminous shale to oxidizing temperatures in the presence of air to reduce its content of sulfidic sulfur below 1.0 per cent by weight, adding basic, slag-forming ingredients to the resulting shale ash in quantity sufficient to produce a basicity in the slag bath corresponding to a content of from about 25 to 45 per cent of CaO, controlling the reducing agent content to a value corresponding to from 1 to 5 times the quantity required for complete reduction of the metal oxides of iron, titanium, vanadium, molybdenum and tungsten mentioned therein, fusing the resulting charge to form a metal bath and a siliceous slag bath, and recovering the slag and the metal.

PER GUNNAR BRUNDELL.

STIG HARALD TJERNSTRÖM.

(References on following page)

## REFERENCES CITED

The following references are of record in the file of this patent:

## UNITED STATES PATENTS

| Number    | Name     | Date          |
|-----------|----------|---------------|
| 1,300,410 | Johnson  | Apr. 15, 1919 |
| 1,334,004 | Toorn    | Mar. 16, 1920 |
| 1,369,298 | Penniman | Feb. 22, 1921 |

| Number      | Name     | Date          |
|-------------|----------|---------------|
| 1,815,888   | Baily    | July 28, 1931 |
| 1,907,868   | Powell   | May 9, 1933   |
| 2,028,105   | Head     | Jan. 14, 1936 |
| 5 2,223,047 | Ramseyer | Nov. 26, 1940 |
| 2,313,044   | Brassert | Mar. 9, 1943  |

## OTHER REFERENCES

Chemical Abstracts, vol. 35, 1941, columns 6397 and 6398, Hultman.